

## 1

3,654,232

**SURFACE BROMINATED FIBERS COMPRISED OF POLY(1,4 - CYCLOHEXYLENE-DIMETHYLENE TEREPHTHALATE)**

Winston J. Jackson, Jr., and John R. Caldwell, Kingsport, Tenn., assignors to Eastman Kodak Company, Rochester, N.Y.

No Drawing. Filed Feb. 5, 1971, Ser. No. 113,029  
Int. Cl. C08g 53/20

U.S. Cl. 260—75 T

4 Claims

**ABSTRACT OF THE DISCLOSURE**

Fibers comprised of poly(1,4-cyclohexylenedimethylene terephthalate) having improved resistance to burning are prepared by contacting the fiber with a brominating agent in the presence of a chlorinating agent, and the sum of bromine and chlorine on the surface of the fiber is at least four percent of the weight of the fiber and the toughness of the fiber is reduced not more than 20 percent, based on the toughness of the fiber before contacting the fiber.

This invention relates to the halogenation of the surface of fibers comprised of poly(1,4-cyclohexylenedimethylene terephthalate) wherein the sum of bromine and chlorine on the surface of the fiber is at least four percent of the weight of the fiber and the toughness of the fiber is reduced not more than 20 percent, based on the toughness of the fiber before contacting the fiber.

Fibers having improved resistance to burning are becoming of increasing importance in numerous applications. The advantages of fire-resistant or self-extinguishing wearing apparel, draperies, rugs, coatings and the like are obvious.

It is well known in the art that halogen can be an effective flame retarder. It is further well known that bromine in many instances is a more effective flame retarder than chlorine. The halogenation of polyester fibers using chlorine and bromine is also known in the art. Specifically, U.S. 2,829,070 to Osborn discloses a process of surface treating, with a mixture of chlorine and bromine, a fiber of a linear polyester, particularly a polyester of terephthalic acid and a glycol selected from the series  $\text{HO}(\text{CH}_2)_n\text{OH}$  wherein  $n$  is an integer from 2-10 inclusive.

We have now found that when the process of Osborn is practiced using a fiber comprised of poly(1,4-cyclohexylenedimethylene terephthalate), the toughness of the fiber is reduced not more than 20 percent based on the toughness of the fiber before contacting the fiber when the sum of bromine and chlorine on the surface of the fiber is at least four percent of the weight of the fiber. These advantageous results are not obtained when the process of Osborn is practiced using the specifically disclosed polyester of terephthalic acid and a glycol selected from the series  $\text{HO}(\text{CH}_2)_n\text{OH}$  wherein  $n$  is an integer from 2-10 inclusive.

Accordingly, it is an advantage of this invention to provide a fiber of improved resistance to burning which has less than 20% reduction in toughness.

Other advantages and features of this invention will be readily apparent to those skilled in the art from the following description and appended claims.

## 2

In broad summary, one embodiment of this invention comprises a process for halogenating the surface of a fiber comprising contacting with a brominating agent in the presence of a chlorinating agent in the temperature range of about 0° C. to about 150° C., a fiber comprised of a highly polymeric linear polyester of

(A) at least 80 mole percent terephthalic acid, and  
(B) at least 80 mole percent 1,4-cyclohexanediethanol,

wherein the sum of bromine and chlorine on the surface of the fiber is at least four percent of the weight of the fiber and the toughness of the fiber is reduced not more than 20 percent, based on the toughness of the fiber before contacting the fiber.

In broad summary, another embodiment of this invention comprises a fiber comprising a highly polymeric linear polyester of

(A) at least 80 mole percent terephthalic acid, and  
(B) at least 80 mole percent 1,4-cyclohexanediethanol,

wherein the sum of bromine and chlorine on the surface of the fiber is at least four percent of the weight of the fiber and the toughness of the fiber is reduced not more than 20 percent, based on the toughness of a similar fiber with no bromine and chlorine on the surface of the fiber.

The preparation of a highly polymeric linear polyester of poly(1,4-cyclohexylenedimethylene terephthalate), as well as the manufacture of fibers comprised thereof, are accomplished according to methods well known in the art. Therefore, these various methods need not be described in detail herein.

As noted earlier, in one embodiment of this invention the fiber is comprised of a polyester of at least 80 mole percent terephthalic acid. In a preferred embodiment the dicarboxylic acid is substantially all terephthalic acid. Dicarboxylic acids that can be used as comonomers with at least 80 mole percent terephthalic acid include aliphatic, alicyclic, and aromatic dicarboxylic acids having up to 40 carbon atoms. Examples of such acids include oxalic, malonic, succinic, adipic, 1,4-cyclohexanedicarboxylic, isophthalic and the like. It will be understood that the corresponding esters of these acids are included in the term "dicarboxylic acid." Copolymers may be prepared using two or more of the above dicarboxylic acids or esters thereof.

Also in one embodiment of this invention the fiber is comprised of a polyester of at least 80 mole percent 1,4-cyclohexanediethanol. In a preferred embodiment the organic diol is substantially all 1,4-cyclohexanediethanol. Organic diols that can be used as comonomers with at least 80 mole percent 1,4-cyclohexanediethanol include aliphatic, alicyclic, and aromatic diols having up to 40 carbon atoms. Examples of some of these diols include ethylene glycol, propylene glycol, butanediol, pentanediol, hexanediol and 1,3-cyclohexanediethanol. Copolymers may be prepared using two or more of the above diols.

The polyesters of this invention have an inherent viscosity of at least 0.5 and preferably at least 0.6 or more measured at 25° C. using 0.23 grams of polymer per 100 ml. of a solvent composed of 60 volumes of phenol and 40 volumes of tetrachloroethane.

In one embodiment of this invention the toughness of the fiber is reduced not more than 20 percent, based on the toughness of the fiber before contacting the

fiber. In another embodiment of this invention the toughness of the fiber is reduced not more than 20 percent, based on the toughness of a similar fiber with no bromine and chlorine on the surface of the fiber.

Toughness is a measure of the area under the stress strain curve. Since this curve is approximately a triangle, toughness in this disclosure and claims is defined as  $\frac{1}{2}$  of the tenacity (in grams per denier) times the elongation (in percent) divided by 100 and is expressed in grams per denier.

Tenacity in this disclosure and claims is a measure of the strength of the fiber and is expressed in grams per denier, abbreviated g./d., and is calculated by dividing the initial denier of the fiber under study into the tension in grams required to break the fiber. The values of tenacity in this disclosure and claims can be determined by using a 5-inch specimen in an Instron Model TM tester at a rate of extension of 100 percent per minute.

Elongation in this disclosure and claims is a measure of the extent to which a fiber is stretched when it breaks. It is expressed as a percentage and is calculated by dividing the original length of the sample into the increase in length and multiplying by 100. It is measured on an Instron Model TM tester by using a 5-inch specimen at a rate of extension of 100 percent per minute.

Although the exact manner in which the surface of the fiber becomes halogenated is not fully understood, one theory suggests the following explanation.

Bromination of polyesters takes place at an appreciably slower rate than chlorination. Our new, improved process consists of carrying out the bromination reaction in the presence of chlorine which, we have found, greatly increases the rate of bromination and the degree of bromination of the polymer. The reason for this, presumably, is because chlorine radicals are more energetic than bromine radicals and react more readily with the polyester to remove a hydrogen atom in the first step of the halogenation mechanism:



wherein R is the remainder of the polyester chain and X<sup>·</sup> is a bromine or chlorine free radical. According to T. L. Cottrell, "The Strengths of Chemical Bonds," 2d edition, Butterworths, London, 1958, the energy required to dissociate a hydrocarbon, R:H, wherein H is a tertiary hydrogen atom is about 89K cal./mole (94K cal./mole for a secondary hydrogen and 100K cal./mole for a primary hydrogen atom); the energy released when the HBr bond is formed is 87K cal./mole, and 102K cal./mole is released when the HCl bond is formed. Consequently, Equation 1 is endothermic when X is bromine and exothermic when X is chlorine. Therefore, it is assumed that this step of the halogenation takes place considerably more readily when X is chlorine. The second step of the halogenation is quite exothermic for both chlorine and bromine:



The bond dissociation energy for bromine is 46K cal./mole, and that for chlorine is 57K cal./mole; the energy released by formation of RBr is about 65K cal./mole, and that for RCl is about 81K cal./mole. Equation 1, therefore, is the rate-determining step.

Since chlorination takes place more readily than bromination, it is necessary to use an excess of bromine, relative to that of chlorine, if bromination is to be the dominant reaction. When a free radical on the polyester chain is produced by chlorine (Equation 1), an excess of bromine over chlorine is present for this radical to react with (Equation 2). Of course some chlorination will also take place, but the amount of such chlorination can be controlled through regulating the bromine to chlorine ratio. That is, if the bromine to chlorine ratio is high, then the rate of bromination that

will occur on the polyester chain will be higher than the chlorination that will occur. Thus, the average molar concentration of bromine to chlorine should be greater than 1:1. Normally, the average molar concentration of bromine should be at least 2 times and preferably at least 3 times that of the chlorine. Formation of the chlorine free radicals to initiate the reaction may be accomplished with visible or ultraviolet radiation, heat, a free radical catalyst, or a combination of these.

10 The polyester fibers may be brominated simply by contacting them with gaseous bromine and chlorine in the presence of visible radiation, ultraviolet radiation, and/or heat for a sufficient time for the desired degree of halogenation to be attained. One process consists of immersing the fibers in bromine water and passing in chlorine while the mixture is heated and/or irradiated with visible or ultraviolet radiation. Instead of water, an organic solvent may be used which will not substantially affect the physical properties of the fibers other than to cause slight swelling. The type of solvent which may be used depends upon the polymer structure. In general, suitable organic solvents include carbon tetrachloride, benzene, and chlorobenzene.

15 The bromination reactions may be carried out at or below room temperature, preferably with the reaction mixtures irradiated with visible or ultraviolet radiation. A more rapid reaction occurs if the mixture is also heated. Temperatures of 0° to 150° C. may be used, depending upon the stability of the polymer, but temperatures of 70° to 120° C. are preferred in aqueous or gaseous systems. The reaction mixture may be heated without illumination with visible or ultraviolet radiation, but a longer reaction time is required.

20 When the bromination is carried out in a liquid medium, the reaction rate may be enhanced by the use of a free radical catalyst or halogenation promoter instead of, or in addition to, heat or illumination. Since the catalyst initiates the free radical reaction by first dissociating into free radicals itself, the catalyst which is used depends upon the reaction temperature, which must be sufficiently high to cause dissociation at a reasonable rate. Examples of suitable free radical catalysts include acetyl peroxide, benzoyl peroxide, lauroyl peroxide, azobisisobutyronitrile, t-butylperoxypivalate, diisopropylperoxydicarbonate, hydrogen peroxide, the alkali metal persulfates and t-butylperoxide.

25 At the conclusion of the bromination, the polyester fibers may be rinsed with water or an organic solvent and dried, or they may be only heated in order to remove liquid and gaseous components from the halogenation reaction. Acetone is a preferred solvent for use in rinsing the polyester fibers.

30 Bromine is the preferred brominating agent, but others may be used under the above reaction conditions in either an aqueous medium or in organic solvents. Examples of other brominating agents include sulfuryl bromide, phosphorus pentabromide, t-butyl hypobromite, sodium hypobromite, potassium hypobromite, and hypobromous acid. Preferably, chlorine gas is used in the process. However, examples of other effective chlorinating agents include sulfuryl chloride, phosphorus pentachloride, t-butyl hypochlorite, sodium hypochlorite, potassium hypochlorite, and hypochlorous acid.

35 The amount of bromine and chlorine which must be substituted on the surface of the fiber in order to make it self-extinguishing depends primarily upon the size of the fiber as the higher denier fibers require more bromine and chlorine to make them self-extinguishing than the lower denier fibers. In general, three denier polyester fibers become self-extinguishing when they contain about four percent bromine, attached substantially on the surface, and they have improved resistance to burning when they contain at least about one percent bromine. In one embodiment of this invention the sum of the chlorine and bromine on the surface of the fiber is at least four per-

cent of the weight of the fiber while in another embodiment the sum of the chlorine and bromine on the surface of the fiber is at least six weight percent of the fiber. In both these embodiments the toughness of the fiber is reduced not more than 20%, based on the toughness of the fiber before contact or based on the toughness of a similar fiber not containing chlorine and bromine on the surface of the fiber.

The fibers which are brominated according to this invention may contain various additives, such as pigments, 10

similarly soaked in acetone. After drying, the inherent viscosity, the amount of chlorine and bromine on the surface of the fiber, based on the weight of the fiber, and the tenacity and elongation are determined for each of the 5 five fiber samples. The toughness, calculated as  $\frac{1}{2}$  the tenacity times the elongation divided by 100, is then calculated and the percent reduction in toughness of the fiber, based on the toughness of the unhalogenated fiber, is calculated. Results of these determinations and calculations are given in Table 1 below.

TABLE I

| Sample Number | Composition                                                                         | Contacting time, min. | Inherent viscosity | Cl, wt. percent | Br, wt. percent | Sum of Cl and Br, wt. percent | Tenacity, g./d. | Elongation, percent | Toughness, g./d. | Reduction in toughness, percent |
|---------------|-------------------------------------------------------------------------------------|-----------------------|--------------------|-----------------|-----------------|-------------------------------|-----------------|---------------------|------------------|---------------------------------|
| 1.....        | Poly(ethylene terephthalate).....                                                   | None                  | 0.59               | None            | None            | None                          | 4.4             | 34                  | 0.75             | .....                           |
|               |                                                                                     | 120                   | 0.21               | 2.9             | 2.5             | 5.4                           | 1.3             | 8                   | 0.05             | 93                              |
| 2.....        | Poly(tetramethylene terephthalate).....                                             | None                  | 0.95               | None            | None            | None                          | 4.4             | 28                  | 0.62             | .....                           |
|               |                                                                                     | 30                    | 0.54               | 1.3             | 3.3             | 4.6                           | 1.6             | 21                  | 0.17             | 72                              |
|               |                                                                                     | 120                   | 0.42               | 4.3             | 5.3             | 9.6                           | 0.3             | 2                   | 0.003            | 99                              |
| 3.....        | Poly(1,4-cyclohexylenedimethylene terephthalate).....                               | None                  | 0.78               | None            | None            | None                          | 3.0             | 18                  | 0.27             | .....                           |
|               |                                                                                     | 15                    | 0.58               | 0.9             | 6.8             | 7.7                           | 2.8             | 20                  | 0.28             | (1)                             |
| 4.....        | Poly(1,4-cyclohexylenedimethylene 80/20 terephthalate/isophthalate).....            | None                  | 0.80               | None            | None            | None                          | 2.8             | 20                  | 0.28             | .....                           |
|               |                                                                                     | 20                    | 0.55               | 1.1             | 9.2             | 10.3                          | 2.5             | 18                  | 0.23             | 18                              |
| 5.....        | Poly(1,4-cyclohexylenedimethylene 90/10 terephthalate/hexahydro-terephthalate)..... | None                  | 0.74               | None            | None            | None                          | 3.0             | 20                  | 0.30             | .....                           |
|               |                                                                                     | 10                    | 0.62               | 0.8             | 5.2             | 6.0                           | 2.9             | 19                  | 0.28             | 7                               |

<sup>1</sup> No reduction.

antioxidants, fire-retardants, and stabilizers. Examples of effective stabilizers include organo-tin sulfur, organo-tin, epoxy, aziridinyl, urea phosphite, unsaturated aliphatic compounds, powdered calcium carbonate, and fatty acid salts of metals, such as cadmium, zinc, and tin.

### EXPERIMENTAL

Experimental work is conducted to demonstrate that when the invention is practiced using fiber comprised of a polyester of terephthalic acid and 1,4-cyclohexanedi-methanol the toughness of the fiber is reduced not more than 20 percent when the sum of the chlorine and bromine on the surface of the fiber is at least four percent of the weight of the fiber, but when the invention is practiced using fibers comprised of a polyester of terephthalic acid and ethylene glycol or terephthalic acid and tetramethyl-ene glycol the same result does not obtain.

In this experimental work a 3-liter, 3-necked flask is equipped with thermometer, gas addition tube, a reflux condenser, and an aluminum foil reflector which is taped to the back side of the flask. Into the flask is then placed 25 ml. of bromine which forms a pool on the bottom of the flask. A 375-watt floodlamp (visible illumination), placed approximately 12 cm. from the flask, is then turned on the flask and the slow addition of chlorine gas is started. After 1 hr., the lamp has increased the temperature in the flask to 105° C.

A first sample of drawn, unheat-set poly(ethylene terephthalate) fiber, a second sample of drawn, unheat-set poly(tetramethylene terephthalate) fiber, a third sample of drawn, unheat-set poly(1,4-cyclohexylenedimethylene terephthalate), a fourth sample of a drawn, unheat-set fiber of 80 mole percent terephthalic acid, 20 mole percent isophthalic acid and 1,4-cyclohexanedi-methanol and a fifth sample of a drawn, unheat-set fiber of 90 mole percent terephthalic acid, 10 mole percent hexahydroterephthalic acid and 1,4-cyclohexanedi-methanol are prepared.

All five of these samples are tied to the blade of a glass stirrer, preheated to 90° C., and placed in the flask through the center neck. The hanks are not allowed to contact the pool of bromine on the bottom of the flask. The stirrer is slowly turned so that all sides of the polyester fiber hanks are equally exposed to the light.

Portions of each of the fiber samples are contacted with bromine in the presence of chlorine for varying lengths of time. When the halogenated fibers are removed from the flask, they are orange in color due to absorbed bromine. To remove this bromine the hanks are soaked in acetone overnight. The unhalogenated controls are 75

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

1460

1465

1470

1475

1480

1485

1490

1495

1500

1505

1510

1515

1520

1525

1530

1535

1540

1545

1550

1555

1560

1565

1570

1575

1580

1585

1590

1595

1600

1605

1610

1615

1620

1625

1630

1635

1640

1645

1650

1655

1660

1665

1670

1675

1680

1685

1690

1695

1700

1705

1710

1715

1720

1725

1730

1735

1740

1745

1750

1755

1760

1765

1770

1775

1780

1785

1790

1795

1800

1805

1810

1815

1820

1825

1830

1835

1840

1845

1850

1855

1860

1865

1870

1875

1880

1885

1890

1895

1900

1905

1910

1915

1920

1925

1930

1935

1940

1945

1950

1955

1960

1965

1970

1975

1980

1985

1990

1995

2000

2005

2010

2015

2020

2025

2030

2035

2040

2045

2050

2055

2060

2065

2070

2075

2080

2085

2090

2095

2100

2105

2110

2115

2120

2125

2130

2135

2140

2145

2150

2155

2160

2165

2170

2175

2180

2185

2190

2195

2200

2205

2210

2215

2220

2225

2230

2235

2240

2245

2250

2255

2260

2265

2270

2275

2280

2285

2290

2295

2300

2305

2310

2315

2320

2325

2330

2335

2340

2345

2350

2355

2360

2365

2370

2375

2380

2385

2390

2395

2400

2405

2410

2415

2420

2425

2430

2435

2440

2445

2450

2455

2460

2465

2470

2475

2480

2485

2490

2495

2500

2505

2510

2515

2520

2525

2530

2535

2540

2545

2550

2555

2560

2565

2570

2575

2580

2585

2590

2595

2600

2605

2610

2615

2620

2625

2630

2635

2640

2645

2650

2655

2660

2665

2670

2675

2680

2685

2690

2695

2700

2705

2710

2715

2720

2725

2730

2735

2740

2745

2750

2755

2760

2765

2770

2775

2780

2785

2790

2795

2800

2805

2810

2815

2820

2825

2830

2835

2840

2845

2850

2855

2860

2865

2870

2875

2880

2885

2890

2895

2900

2905

2910

2915

2920

2925

2930

2935

2940

2945

2950

2955

2960

2965

2970

2975

2980

2985

2990

2995

3000

3005

3010

3015

3020

3025

3030

3035

3040

3045

3050

3055

3060

3065

3070

3075

3080

3085

3090

3095

3100

3105

3110

3115

3120

3125

3130

3135

3140

3145

3150

3155

3160

3165

3170

3175

3180

3185

3190

3195

3200

3205

3210

3215

3220

3225

3230

3235

3240

3245

3250

3255

3260

3265

3270

3275

3280

3285

3290

3295

3300

3305

3310

3315

3320

3325

3330

3335

3340

3345

3350

3355

3360

3365

3370

3375

3380

3385

3390

3395

3400

3405

3410

3415

3420

3425

3430

3435

3440

3445

3450

3455

3460

3465

3470

3475

3480

3485

3490

3495

3500

3505

3510

3515

3520

3525

3530

3535

3540

3545

3550

3555

3560

3565

3570

3575

3580

3585

3590

3595

3600

3605

3610

3615

3620

3625

3630

3635

3640

3645

3650

3655

3660

3665

3670

3675

3680

3685

3690

3695

3700

3705

3710

3715

3720

3725

3730

3735

3740

3745

3750

3755

3760

3765

3770

3775

3780

3785

3790

3795

3800

3805

3810

3815

3820

3825

3830

3835

3840

3845

3850

3855

3860

3865

3870

3875

3880

3885

3890

3895

3900

3905

3910

3915

3920

3925

3930

3935

3940

3945

3950

3955

3960

3965

3970

3975

3980

3985

3990

3995

4000

4005

4010

4015

4020

4025

4030

4035

4040

4045

4050

4055

4060

4065

4070

4075

4080

4085

4090

4095

4100

4105

4110

4115

4120

4125

4130

4135

4140

4145

4150

4155

4160

4165

4170

4175

4180

4185

4190

4195

4200

4205

4210

4215

4220

4225

4230

4235

4240

4245

4250

4255

4260

4265

4270

4275

4280

4285

4290

4295

4300

4305

4310

4315

4320

4325

4330

4335

4340

4345

4350

4355

4360

4365

4370

4375

4380

4385

4390

4395

4400

4405

4410

4415

4420

4425

4430

4435

4440

4445

4450

4455

4460

4465

4470

4475

4480

4485

4490

4495

4500

4505

4510

4515

4520

4525

4530

4535

4540

4545

4550

4555

4560

4565

4570

4575

4580

4585

4590

4595

4600

4605

4610

4615

4620

4625

4630

4635

4640

4645

4650

4655

4660

4665

4670

4675

4680

4685

4690

4695

4700

4705

4710

4715

4720

4725

4730

4735

4740

4745

4750

4755

4760

4765

4770

4775

4780

4785

4790

4795

4800

4805

4810

4815

4820

4825

4830

4835

4840

4845

4850

4855

4860

4865

4870

4. The fiber of claim 3 wherein a halogenation promoter is added to the process, the halogenation promoter being selected from the group consisting of acetyl peroxide, benzoyl peroxide, lauroyl peroxide, azobisisobutyronitrile, t-butylperoxy pivalate, di-isopropylperoxydicarbonate, hydrogen peroxide, the alkali metal persulfates, and t-butylperoxide.

|             |         |                       |          |
|-------------|---------|-----------------------|----------|
| 2,702,283   | 2/1955  | Wilson et al. -----   | 260—6    |
| 2,754,217   | 7/1956  | Allen et al. -----    | 106—15   |
| 2,755,260   | 7/1956  | Stilbert et al. ----- | 260—17.4 |
| 2,829,070   | 4/1958  | Osborn -----          | 117—93   |
| 5 3,274,163 | 9/1966  | Elfers et al. -----   | 260—78.4 |
| 3,285,995   | 11/1966 | Nametz et al. -----   | 260—865  |
| 3,356,631   | 12/1967 | Jackson et al. -----  | 260—31.2 |
| 3,454,672   | 7/1969  | Jackson et al. -----  | 260—860  |

## References Cited

## UNITED STATES PATENTS

2,607,802 8/1952 Britton et al. ----- 260—544  
2,658,086 11/1953 Ruh et al. ----- 260—653

10 MELVIN GOLDSTEIN, Primary Examiner

U.S. Cl. X.R.

260—75 H